

K. TORNBERG.

ELECTRODE.

APPLICATION FILED AUG. 28, 1918.

1,334,820.

Patented Mar. 23, 1920.

Fig. 1.



Fig. 2.



Inventor:  
Knut Tornberg,  
by *A. Knut G. Davis*  
His Attorney.

# UNITED STATES PATENT OFFICE.

KNUT TORNBERG, OF LYNN, MASSACHUSETTS, ASSIGNOR TO GENERAL ELECTRIC COMPANY, A CORPORATION OF NEW YORK.

## ELECTRODE.

1,334,820.

Specification of Letters Patent. Patented Mar. 23, 1920.

Application filed August 28, 1918. Serial No. 251,848.

To all whom it may concern:

Be it known that I, KNUT TORNBERG, a citizen of the United States, residing at Lynn, in the county of Essex, State of Massachusetts, have invented certain new and useful Improvements in Electrodes, of which the following is a specification.

My invention has reference to improvements in negative electrodes used in connection with positive electrodes of copper or other metals or combinations of metals which are generally spoken of as non-consuming electrodes, while the negatives are consumed at a rate depending on the type used and strength of current. The principal ingredient of the negative electrodes is an iron oxid, mainly the magnetic oxid of iron called magnetite ( $Fe_3O_4$ ), and these electrodes are, therefore, known in the art as magnetite electrodes. Various admixtures are used with the magnetite; some native or artificial materials containing titanium and some containing chromium. The principal titanium bearing materials used either singly or in combination as admixtures to the magnetite are rutile, ilmenite and titanium carbid, and in addition to these are used minute quantities of various fluxes, such, for example, either singly or in combination the fluorids of sodium, potassium, lithium, magnesium and calcium, as well as other compounds.

It has been found that magnetite mixtures in which ilmenite is used in place of the more expensive rutile while working successfully with such low current as 4 amperes exhibit one defect when operated with currents as high as 6.6 amperes, which are carried on many arc lamp circuits. When run at this higher current (6.6 amps.) these electrodes form at the arcng end a cap which does not securely fuse to the iron tube in which the mixture is held; the caps become loose and by the operation of starting and feeding they are knocked off, and have to be formed anew so frequently that at this higher current these electrodes could not be commercially used.

Another defect in which all magnetite electrodes share (whether of the rutile or ilmenite type) is the formation at the arcng end of a liquid pool. This is called "puddling" of the electrode and it gives rise to rotation of the arc with consequent unsteadiness of the light. The usual means

for overcoming puddling is the addition to the electrode mixture of one or more of the fluxes heretofore mentioned; but some of these fluxes depress the candle power, some increase consumption, while some have other drawbacks, as for example, that of being expensive.

By my invention puddling is cured simply, cheaply and effectively, and by its use ilmenite becomes available in place of rutile for magnetite electrodes and can be operated at the higher current.

The invention consists in the application to the inner wall of the iron electrode tube of a film of water-glass, either the potassium or the sodium silicate.

The accompanying drawing shows in Figure 1, a longitudinal axial section of a magnetite electrode embodying my invention, and in Fig. 2 a like section of the upper part of a modification thereof.

Referring to Fig. 1, the electrode tube 1, usually made of iron, is closed at the bottom by a thimble 2, and the inner surface of the tube is lined with a film 3 of water-glass. This water-glass may be either the silicate of potassium or the silicate of soda, or a mixture of both. Each of these ingredients, used alone, has proved to be quite effective for the purposes of my invention. The film may be applied by flooding the inner surface of the tube with an aqueous solution of the water-glass and allowing the same to drain and dry. Of course, any other method of producing a thin coating of water-glass may be used.

The magnetite mixture 4 is then filled into and compacted in the tube, is then topped with a seal 6 about  $\frac{1}{8}$ " thick, consisting of filling mixture made into a plastic mass by shellac solution and the tube is then closed by a metal disk 5, as usual.

This film of water glass causes the cap formation to fuse securely to the iron shell of the electrode. It also prevents puddling without the use of fluxes, which heretofore have been found necessary for this purpose. It is the immediate contiguity of the requisite amount of water glass both to the magnetite mixture and to the iron shell that renders the fusion of the cap formation to the shell a matter of certainty throughout the length of the electrode. A like certainty of the fusion of the cap to the shell cannot be attained when the water glass is made a

part of the filling mixture, no matter how uniformly it may be distributed throughout the mass. This is due to the fact that the water glass particles remote from the wall 5 of the shell do not, or do not directly participate in the fusion process.

With my invention applied the addition of a flux or fluxes to the magnetite mixture may be (and should be) dispensed with in 10 the filling mixture proper.

But in the case of so-called "high efficiency" mixtures, *i. e.* magnetite mixtures referred to above as being of the rutile type and containing titanium carbide besides the 15 rutile, I have found it desirable, even though not absolutely necessary, to use a special seal immediately beneath the capping disk 5. This is shown in Fig. 2, the special seal consisting of a layer 6' about  $\frac{1}{4}$ " thick, of filling 20 mixture into which has been incorporated about one-half of one per cent. of anhydrous potassium fluorid, shellac solution being used as a binder, as in the case of the usual seal, mentioned above; the special seal thus 25 becomes a solidified button.

This special seal 6' acts as an additional insurance against puddling to which these

high efficiency electrodes are especially prone during the first few hours of their life, the salutary effect of the minute quantity of potassium fluorid contained in the special seal apparently persisting long after the special seal itself has been consumed.

What I claim as new and desire to secure by Letters Patent of the United States, is:— 3

1. An electrode comprising a metal tube, 3 a film of water-glass on the inner surface thereof, and a filling of a magnetite mixture in the tube.

2. An electrode comprising a metal tube, 4 a film of water-glass on the inner surface thereof, and a filling of ilmenite in the tube.

3. An electrode comprising a metal tube, 4 a film of water-glass on the inner surface thereof, a filling of a magnetite mixture in the tube, and a seal on top of the filling, consisting of a solidified button of plastic filling material, having about one-half of one per cent. of anhydrous potassium fluorid incorporated therein. 5

In witness whereof, I have hereunto set my hand this 26th day of August, 1918.

KNUT TORNBERG.